

Patented Dec. 20, 1927.

1,653,605

## UNITED STATES PATENT OFFICE.

EDGAR ARTHUR ASHCROFT, OF WAYE, NEAR ASHBURTON, ENGLAND, ASSIGNOR TO  
NEW METALLURGY LIMITED, OF LONDON, ENGLAND, AN INCORPORATED ENGLISH  
JOINT-STOCK COMPANY.

METHOD OF PROTECTING CARBON OR GRAPHITE ELECTRODES IN FUSED ELECTROLYTES.

No Drawing. Application filed February 23, 1927, Serial No. 170,412, and in Great Britain November 27, 1925.

The present invention relates to improvements in the operation of electrolytic cells employing fused electrolytes, and refers more particularly to the protection of the 5 carbon or graphite electrodes from the action of moisture and/or oxygen which normally cause destruction of the said electrodes.

According to the present invention, in an 10 electrolytic process using a fused electrolyte and wherein one or more carbon or graphite electrodes are employed, I provide a method of protecting said electrodes against attack by oxygen, said method consisting in the introduction of sulphur or a 15 sulphur compound or mixture into the electrolyte or onto the surface thereof in quantity sufficient to ensure the combination with sulphur of the whole of the oxygen present 20 in the electrolyzer. In this manner the destruction of the electrodes by oxidation is prevented, the protection extending both to the parts of the electrodes immersed in the electrolyte and in the gas space above the 25 electrolyte. Normally the presence of air in this space burns away the carbon or graphite electrodes due to the high operating temperature of the electrolyzer. On the addition of sulphur, however, the latter 30 burns first by reason of lower ignition temperature. In the electrolyte any oxygen compound which may be present is decomposed and the oxygen instead of attacking the electrodes combines with the sulphur. 35 The invention is applicable to electrolytic processes in general in which the fused salts of metals are electrolyzed for the recovery of the metal, and in which normally little or no sulphur or incompletely oxidized sulphur 40 compounds are present.

It has, however, an especially valuable commercial application in the electrolytic recovery of zinc and lead from fused baths of their chlorides.

45 In this case the action of the sulphur in protecting the plates appears to be to form various compounds such as  $SO_2$ ,  $SO_2Cl_2$  and  $S(OH)Cl$  none of which oxidizes the graphite plates at the temperature working of the 50 electrolyzer, whereas oxygen compounds

which are decomposed yielding oxygen at the anode in the absence of sulphur are highly destructive.

Instead of introducing sulphur I may introduce sulphur chloride to the electrolyzer 55 in liquid form for a similar purpose or I may introduce any suitable sulphide—such as lead sulphide—when the electrolyzer is producing lead—or zinc sulphide—when the electrolyzer is producing zinc. The sulphide will then be decomposed the metal 60 going to the cathode and the resulting sulphur acting as above described with the anode product.

I may vary the above described process 65 by introducing small quantities of sulphates in conjunction with sulphides or sulphur or of sulphites or even of oxides—provided an excess of sulphur is present also—the necessary conditions being that the total amount 70 of sulphur present shall always be sufficient to prevent the liberation of free oxygen at the anode surfaces, and also that nothing but one or other of the above described compounds or analogous compounds which do 75 not oxidize or act detrimentally on the anodes will be formed. It is then found that there is no attack on the graphite plates even if moist air be introduced to the electrolyzer. Without such precautions as above described 80 the introduction of moist air to an electrolyzer brings about destruction of the plates.

In carrying out this invention it will be apparent that it is advisable to maintain the sulphur, in whatever form it is added, in 85 some excess of such oxygen as may be present in or enter the electrolyzer.

What I claim is:

1. In an electrolytic process using a fused electrolyte and wherein a carbon or graphite electrode is employed, a method of protecting said electrode against attack by oxygen consisting in the introduction of sulphur to the electrolyzer in quantity approximately only sufficient to ensure the combination with sulphur of the whole of the oxygen present in the electrolyzer.

2. In an electrolytic process using a fused electrolyte and wherein a carbon or graphite electrode is employed, a method of pro-

protecting said electrode against attack by oxygen, consisting in the introduction of a sulphur compound to the electrolyzer in quantity approximately only sufficient to ensure 5 the combination with sulphur of the whole of the oxygen present in the electrolyzer.

3. In an electrolytic process using a fused electrolyte and wherein a carbon or graphite electrode is employed, a method of protecting 10 said electrode against attack by oxygen, consisting in the introduction of metallic sulphides in the electrolyzer in quantity approximately only sufficient to ensure the

combination with sulphur of the whole of the oxygen present in the electrolyzer. 15

4. In an electrolytic process using a fused electrolyte and wherein a carbon or graphite electrode is employed, a method of protecting said electrode against attack by oxygen, consisting in the introduction of the sulphide of the metal which is being recovered to the electrolyzer in quantity approximately only sufficient to ensure the combination with sulphur of the whole of the oxygen present in the electrolyzer. 20

EDGAR ARTHUR ASHCROFT.